



US010472730B2

(12) **United States Patent**  
Mayer et al.

(10) **Patent No.:** US 10,472,730 B2  
(45) **Date of Patent:** Nov. 12, 2019

(54) **ELECTROLYTE CONCENTRATION  
CONTROL SYSTEM FOR HIGH RATE  
ELECTROPLATING**

(71) Applicant: **Novellus Systems, Inc.**, Fremont, CA (US)

(72) Inventors: **Steven T. Mayer**, Aurora, OR (US); **Jonathan David Reid**, Sherwood, OR (US); **Seshasayee Varadarajan**, Lake Oswego, OR (US)

(73) Assignee: **Novellus Systems, Inc.**, Fremont, CA (US)

(\*) Notice: Subject to any disclaimer, the term of this patent is extended or adjusted under 35 U.S.C. 154(b) by 174 days.

(21) Appl. No.: **14/800,344**

(22) Filed: **Jul. 15, 2015**

(65) **Prior Publication Data**

US 2015/0315720 A1 Nov. 5, 2015

**Related U.S. Application Data**

(63) Continuation-in-part of application No. 12/577,619, filed on Oct. 12, 2009, now Pat. No. 9,109,295.

(51) **Int. Cl.**

**C25D 21/18** (2006.01)

**C25D 7/12** (2006.01)

**C25D 3/38** (2006.01)

(52) **U.S. Cl.**

CPC ..... **C25D 21/18** (2013.01); **C25D 3/38** (2013.01); **C25D 7/123** (2013.01)

(58) **Field of Classification Search**

CPC ..... C25D 21/18

See application file for complete search history.

(56)

**References Cited**

U.S. PATENT DOCUMENTS

H000036 H 3/1986 Smith  
5,391,271 A \* 2/1995 Ludwig ..... G01N 27/42  
204/434

(Continued)

FOREIGN PATENT DOCUMENTS

CN 1303124 A 7/2001  
CN 1506499 A 6/2004

(Continued)

OTHER PUBLICATIONS

Xiao et al., "Preparation and Performance of Shape Stabilized Phase Change Thermal Storage Materials with High Thermal Conductivity" Ener. Conv. Manage. 43(1), pp. 103-108 (2002).\*

(Continued)

*Primary Examiner* — Bryan D. Ripa

(74) *Attorney, Agent, or Firm* — Weaver Austin Villeneuve & Sampson LLP

(57) **ABSTRACT**

An electroplating apparatus for filling recessed features on a semiconductor substrate includes a vessel configured to maintain a concentrated electroplating solution at a temperature of at least about 40° C., wherein the solution would have formed a precipitate at 20° C. This vessel is in fluidic communication with an electroplating cell configured for bringing the concentrated electrolyte in contact with the semiconductor substrate at a temperature of at least about 40° C., or the vessel is the electroplating cell. In order to prevent precipitation of metal salts from the electrolyte, the apparatus further includes a controller having program instructions for adding a diluent to the concentrated electroplating solution in the vessel to avoid precipitation of a salt from the concentrated electroplating solution in response to a signal indicating that the electrolyte is at risk of precipitation.

**15 Claims, 9 Drawing Sheets**



|      |                          |                          |             |                 |         |
|------|--------------------------|--------------------------|-------------|-----------------|---------|
| (56) | <b>References Cited</b>  |                          | KR          | 10-2002-0077811 | 10/2002 |
|      | U.S. PATENT DOCUMENTS    |                          | TW          | 200532057 A     | 10/2005 |
|      | 5,425,862 A *            | 6/1995 Hartmann .....    | C25D 7/0614 | 200633032 A     | 9/2006  |
|      |                          |                          | WO          | WO 2010/022009  | 2/2010  |
|      | 5,858,196 A              | 1/1999 Ikenaga           |             |                 |         |
|      | 6,113,771 A              | 9/2000 Landau et al.     |             |                 |         |
|      | 6,231,743 B1             | 5/2001 Etherington       |             |                 |         |
|      | 6,261,433 B1             | 7/2001 Landau            |             |                 |         |
|      | 6,350,366 B1             | 2/2002 Landau et al.     |             |                 |         |
|      | 6,527,920 B1 *           | 3/2003 Mayer .....       | C25D 21/12  |                 |         |
|      |                          |                          | 204/237     |                 |         |
|      | 6,576,111 B1             | 6/2003 Hupe et al.       |             |                 |         |
|      | 7,264,704 B2 *           | 9/2007 Nevosi .....      | C25D 21/18  |                 |         |
|      |                          |                          | 204/237     |                 |         |
|      | 7,405,157 B1             | 7/2008 Reid et al.       |             |                 |         |
|      | 7,670,950 B2             | 3/2010 Richardson et al. |             |                 |         |
|      | 7,776,741 B2             | 8/2010 Reid et al.       |             |                 |         |
|      | 8,043,967 B2             | 10/2011 Reid et al.      |             |                 |         |
|      | 8,128,791 B1 *           | 3/2012 Buckalew .....    | C25D 17/002 |                 |         |
|      |                          |                          | 204/237     |                 |         |
|      | 8,722,539 B2             | 5/2014 Reid et al.       |             |                 |         |
|      | 9,109,295 B2             | 8/2015 Reid et al.       |             |                 |         |
|      | 2003/0079683 A1          | 5/2003 Nakano et al.     |             |                 |         |
|      | 2003/0106802 A1          | 6/2003 Hagiwara et al.   |             |                 |         |
|      | 2003/0186540 A1          | 10/2003 Ito et al.       |             |                 |         |
|      | 2004/0022940 A1          | 2/2004 Nagai et al.      |             |                 |         |
|      | 2004/0134682 A1          | 7/2004 En et al.         |             |                 |         |
|      | 2004/0154917 A1          | 8/2004 Ishida            |             |                 |         |
|      | 2005/0000814 A1          | 1/2005 Metzger           |             |                 |         |
|      | 2005/0241946 A1          | 11/2005 Nagai et al.     |             |                 |         |
|      | 2006/0144699 A1 *        | 7/2006 Klocke .....      | C25D 21/18  |                 |         |
|      |                          |                          | 204/228.6   |                 |         |
|      | 2007/0158202 A1 *        | 7/2007 Nagai .....       | C25D 21/14  |                 |         |
|      |                          |                          | 205/101     |                 |         |
|      | 2007/0187237 A1          | 8/2007 San et al.        |             |                 |         |
|      | 2007/0235341 A1          | 10/2007 Mizohata et al.  |             |                 |         |
|      | 2007/0235392 A1 *        | 10/2007 Edwards .....    | B01F 3/088  |                 |         |
|      |                          |                          | 210/739     |                 |         |
|      | 2009/0038947 A1          | 2/2009 Dubin et al.      |             |                 |         |
|      | 2010/0041226 A1          | 2/2010 Reid et al.       |             |                 |         |
|      | 2010/0200412 A1          | 8/2010 Reid et al.       |             |                 |         |
|      | 2011/0083965 A1 *        | 4/2011 Reid .....        | C25D 3/38   |                 |         |
|      |                          |                          | 205/101     |                 |         |
|      | 2011/0266154 A1 *        | 11/2011 Pavlov .....     | C25D 21/12  |                 |         |
|      |                          |                          | 205/81      |                 |         |
|      | 2012/0031768 A1          | 2/2012 Reid et al.       |             |                 |         |
|      | FOREIGN PATENT DOCUMENTS |                          |             |                 |         |
| CN   | 1610066 A                | 4/2005                   |             |                 |         |
| CN   | 1679154 A                | 10/2005                  |             |                 |         |
| CN   | 1773675 A                | 5/2006                   |             |                 |         |
| CN   | 101022703 A              | 8/2007                   |             |                 |         |
| CN   | 101622585 A              | 1/2010                   |             |                 |         |
| CN   | 202465938 U              | 10/2012                  |             |                 |         |
| CN   | 102995096 A              | 3/2013                   |             |                 |         |
| CN   | 103035544 A              | 4/2013                   |             |                 |         |
| CN   | 104060319 A              | 9/2014                   |             |                 |         |
| JP   | 09-223858                | 8/1997                   |             |                 |         |
| JP   | 2003-113479              | 4/2003                   |             |                 |         |
| KR   | 10-1999-0015599          | 3/1999                   |             |                 |         |

\* cited by examiner



*Figure 1A*



*Figure 1B*



*Figure 1C*

*Figure 2A*



*Figure 2B*



Figure 2C



Figure 3



*Figure 4*



Figure 5



Figure 6



Figure 7

## ELECTROLYTE CONCENTRATION CONTROL SYSTEM FOR HIGH RATE ELECTROPLATING

### CROSS REFERENCE TO RELATED PATENT APPLICATION

This application is a continuation-in-part claiming priority to U.S. patent application Ser. No. 12/577,619 filed Oct. 12, 2009, titled “Electrolyte Concentration Control System for High Rate Electroplating” naming Reid et al. as inventors, which is herein incorporated by reference in its entirety and for all purposes.

### FIELD OF THE INVENTION

The present invention relates generally to methods and apparatus for electrodepositing metals on semiconductor substrates having recessed features and more particularly to methods and apparatus for electroplating copper for filling through silicon vias (TSVs).

### BACKGROUND OF THE INVENTION

A TSV is a vertical electrical connection passing completely through a silicon wafer or die. TSV technology is important in creating 3D packages and 3D integrated circuits (IC). It provides interconnection of vertically aligned electronic devices through internal wiring that significantly reduces complexity and overall dimensions of a multi-chip electronic circuit.

A typical TSV process involves forming TSV holes and depositing conformal diffusion barrier and conductive seed layers, followed by filling of TSV holes with a metal. Copper is typically used as the conductive metal in TSV fill as it supports high current densities experienced at complex integration, such as 3D packages and 3D integrated circuits, and increased device speed. Furthermore, copper has good thermal conductivity and is available in a highly pure state.

TSV holes typically have high aspect ratios making void-free deposition of copper into such structures a challenging task. CVD deposition of copper requires complex and expensive precursors, while PVD deposition often results in voids and limited step coverage. Electroplating is a more common method of depositing copper into TSV structures; however, electroplating also presents a set of challenges because of the TSV’s large size and high aspect ratio.

In a typical TSV electrofilling process, the substrate is contacted with a plating solution which includes copper sulfate as a source of copper ions, sulfuric acid for controlling conductivity, chloride ion to enhance suppressor adsorption and several other additives. However, the use of standard commercially available electrolytes often results in very slow plating and in formation of voids during TSV filling. For example, a typical electrolyte is prepared by combining a solution of copper sulfate, which is supplied at  $\text{Cu}^{2+}$  concentration of less than 65 g/L with concentrated or 50% concentrated sulfuric acid. Pre-mixed electrolytes containing both copper salt and an acid are also available, however they typically have  $\text{Cu}^{2+}$  concentrations of less than 60 g/L. In both cases, the commercially available solutions are prepared at such concentrations so as to avoid precipitation of copper salts at shipping and storage temperature of between about 0-10° C.

### SUMMARY

It is herein provided that the use of commercially available electrolytes which are unsaturated at 0° C., results in

plating rates which may be unacceptably slow (e.g., an hour or more for TSV fill), and may also be associated with increased formation of voids during TSV filling.

The present invention, in one aspect, provides methods and associated apparatus for filling TSVs at very high rates. In some embodiments, this involves using an electrolyte, which has a very high concentration of  $\text{Cu}^{2+}$  ions, typically significantly higher than concentrations provided by commercially available electrolytes. In some embodiments, the 10 electrolyte further includes an acid (e.g., sulfuric acid, an alkylsulfonic acid, mixtures of acids, etc.) at a relatively high concentration, such as at a concentration of between about 0.1-2M. In some embodiments the concentration of acid of at least about 0.6 M is preferred. For example, in 15 some embodiments, the electrolyte contains sulfuric acid at a concentration of between about 40-200 g/L, such as between about 100-200 g/L, preferably at least about 60 g/L.

Further, in many embodiments, electroplating with this 20 concentrated electrolyte is performed at elevated temperatures, such as at least at about 40° C. In some embodiments, electroplating is performed using an electrolyte solution that would have been beyond its saturation limit (i.e., would have 25 formed a precipitate) at a first temperature, wherein the electroplating is performed at a temperature that is at least 10° C. or 20° C. higher than the highest temperature at which the electrolyte is saturated. For example, in some embodiments, electroplating is performed at a temperature of at least about 20° C. with an electrolyte solution which would have formed a precipitate at 0° C. In other embodiments, 30 electroplating is performed at a temperature of at least about 40° C. with a concentrated electrolyte solution, which would have formed a precipitate at 20° C.

In another aspect, the present invention provides an 35 apparatus and associated methods for preparing such concentrated electrolytes prior to use, and for integrating concentrated electrolyte preparation modules with an electroplating apparatus. Further, methods and apparatus for controlling electrolyte concentrations and temperatures are 40 provided. Provided methods and apparatus are particularly useful for filling large high aspect ratio features, such as TSVs with copper, but are also generally applicable for depositing other metals on a variety of semiconductor substrates having recessed features.

In one embodiment an electroplating apparatus for depositing 45 copper on a semiconductor substrate having one or more recessed features (such as TSVs) is provided. The apparatus includes (a) an electrolyte concentrator module configured for concentrating an electrolyte comprising a copper salt, the electrolyte concentrator module comprising an inlet port configured for receiving a non-concentrated electrolyte from a source of non-concentrated electrolyte, an outlet port configured for delivering warm concentrated electrolyte to a concentrated electrolyte reservoir, and a heater configured for maintaining the electrolyte in the 50 concentrator module at a temperature of at least about 40° C.; (b) the concentrated electrolyte reservoir in fluidic communication with the concentrator module, wherein the reservoir is configured for receiving the warm concentrated electrolyte from the concentrator module and for delivering the warm concentrated electrolyte to an electroplating cell; and (c) the electroplating cell in fluidic communication with the concentrated electrolyte reservoir, wherein the electroplating cell is configured for receiving the warm concentrated electrolyte from the concentrated electrolyte reservoir, 55 and for bringing the warm concentrated electrolyte in contact with the semiconductor substrate at the electrolyte temperature of at least about 40° C. (e.g., of at least about 60

50° C., such as of at least about 60° C.). In some embodiments, the apparatus also includes a source of non-concentrated electrolyte in fluidic communication with the concentrator module, wherein the source of non-concentrated electrolyte is configured for holding the non-concentrated electrolyte and for delivering the non-concentrated electrolyte to the inlet port of the concentrator module.

The concentrator module of the electroplating apparatus is configured for removing water from the non-concentrated electrolyte (e.g., by evaporation at elevated temperature and/or by reverse osmosis). For example, in one embodiment, the concentrator is configured for removing water from the non-concentrated electrolyte to form the warm concentrated electrolyte having a temperature of at least about 40° C., wherein the formed warm concentrated electrolyte would have been supersaturated (would have formed precipitate) at 20° C. The concentrator module typically comprises a heater which is electrically connected to a temperature controller, which is configured to maintain the electrolyte temperature in the concentrator module at least at about 40° C. In some embodiments, the concentrator is configured for evaporating water from electrolyte at a temperature of at least about 70° C. In some embodiments, the concentrator is equipped with an inlet configured for receiving dry air and an outlet configured for removing wet air, while the concentrator is working.

The concentrator module further can include a concentration detector (e.g., an optical detector) connected with a concentration controller configured to maintain electrolyte concentration in the desired range. The electrolyte in the concentrator module typically includes  $\text{Cu}^{2+}$  and  $\text{SO}_4^{2-}$  ions,  $\text{H}^+$  (acid),  $\text{Cl}^-$  (chloride), but may also include other components. In one embodiment, the concentrator is configured to concentrate a solution consisting essentially of water with  $\text{Cu}^{2+}$ ,  $\text{SO}_4^{2-}$  (including associated sulfur-containing anions),  $\text{H}^+$ , and  $\text{Cl}^-$  dissolved therein. The concentrator may further include a diluent port configured for receiving a diluent (e.g., DI water) from a diluent source, for example when concentration of electrolyte starts exceeding the desired concentration, and to prevent (or reverse) precipitation of copper salts.

In some embodiments, the concentrator module comprises a recirculation line connected to the electrolyte outlet port, wherein the line is configured for recirculating the warm concentrated electrolyte within the concentrator module and comprising a filter configured for filtering the recirculated electrolyte, wherein the recirculation line is in fluidic communication with the concentrated electrolyte reservoir, and is further configured for delivering the warm filtered concentrated electrolyte to the concentrated electrolyte reservoir.

After the concentrated electrolyte solution (which often has a  $\text{Cu}^{2+}$  concentration of 85 g/L and more) is formed in the concentrator module, it is directed to a concentrated electrolyte reservoir. The reservoir typically also comprises a heater which is electrically connected to a temperature controller, which is configured to maintain the electrolyte temperature in the reservoir at least at about 40° C. The electrolyte temperatures in the concentrator module and in the reservoir need not necessarily be identical, with concentrator electrolyte temperature often being higher than electrolyte temperature in the reservoir. In each case, the temperatures and electrolyte concentrations are judiciously controlled, such that no precipitation from the concentrated solution is occurring. In some embodiments, the reservoir also includes a diluent port configured to deliver a diluent into the reservoir in order to prevent or reverse copper salt

precipitation, or in order to optimize copper concentration in electrolyte solution. Further, in some embodiments the reservoir includes an additive port, which is configured to deliver additives, such as levelers, accelerators, and suppressors to the reservoir from an additive source.

After the concentrated electrolyte leaves the reservoir, it is directed to the plating cell where it is brought in contact with the substrate at a temperature of at least about 40° C., and where electrodeposition occurs. In one embodiment, the 10 warm concentrated electrolyte is delivered continuously to the plating cell through an electrolyte entry port, and is removed through an electrolyte exit port. In some embodiments, the exiting electrolyte is directed through a recirculation line back to the concentrated electrolyte reservoir. 15 Typically, there is a filter in the electrolyte recirculation loop which is adapted for removing insoluble matter from the electrolyte before it re-enters the reservoir. In other embodiments, the exiting electrolyte from the plating cell is directed to the concentrator module through the recirculation line.

20 In another aspect, the concentrated electrolyte is prepared by combining a concentrated solution of copper salt with a solution of acid. In one embodiment the electroplating apparatus includes (a) a concentrated electrolyte reservoir in fluidic communication with a source of concentrated copper salt and with a separate source of a concentrated acid, the reservoir configured for combining the concentrated solution of copper salt with the concentrated acid and forming a warm concentrated electrolyte solution having a temperature of at least about 40° C., wherein the solution would have 25 formed a precipitate at 20° C.; and (b) an electroplating cell in fluidic communication with the concentrated electrolyte reservoir, wherein the electroplating cell is configured for receiving the warm concentrated electrolyte from the concentrated electrolyte reservoir, and for bringing the warm concentrated electrolyte in contact with the semiconductor substrate at the electrolyte temperature of at least about 40° C.

As it was mentioned above, while in many embodiments it is preferable to perform electroplating with concentrated electrolytes above room temperature, in some embodiments concentrated electroplating solutions which would have been supersaturated at 0° C. are prepared, and the plating is performed at 20° C. and above (but not necessarily above room temperature). In one aspect, the plating method for 40 filling a TSV includes: (a) providing a non-concentrated electrolyte solution comprising at least one copper salt, wherein said solution is not saturated at 0° C. and at higher temperatures; (b) concentrating the non-concentrated electrolyte solution comprising said at least one copper salt to 45 form a concentrated solution and maintaining said concentrated solution at a temperature of at least about 20° C., wherein said concentrated solution would have formed a precipitate at 0° C.; and (c) contacting the semiconductor substrate with the concentrated electrolyte solution at a 50 temperature of at least about 20° C. in an electroplating apparatus to at least partially fill the through-silicon via with copper.

In another embodiment the method of TSV filling involves (a) forming a concentrated electrolyte solution by 55 combining a concentrated solution comprising a copper salt with a concentrated solution of acid, said acid having the same anion as the copper salt, to form a concentrated electrolyte solution, wherein said concentrated solution would have formed a precipitate at 0° C., and wherein the formed concentrated solution is maintained at a temperature of at least about 20° C.; and (b) contacting the semiconductor substrate with the concentrated electrolyte solution at a

temperature of at least about 20° C. in an electroplating apparatus to at least partially fill the through-silicon via with copper.

Of course, in some embodiments, the concentrated electrolyte is prepared at least at about 40° C. and is brought in contact with the substrate at least at about 40° C. The concentration of Cu<sup>2+</sup> in the formed concentrated electrolyte will depend on the saturation requirements for a particular electrolyte composition at 0° C. For example, when electrolytes having high concentration of common anion are used, such as copper sulfate electrolyte having high concentration of sulfuric acid, electrolytes with Cu<sup>2+</sup> concentrations of 40 g/L and above may be already supersaturated at 0° C. Such electrolytes would be difficult to obtain, unless methods described herein are used. Thus, in some embodiments, electrolytes having Cu<sup>2+</sup> concentration of 40 g/L and higher, such as 60 g/L and higher, such as 85 g/L and higher are formed. For electrolytes that do not include high concentrations of common anion, supersaturation at 0° C. can be achieved at Cu<sup>2+</sup> concentrations of 85 g/L and above.

These and other features and advantages of the present invention will be described in more detail with reference to the figures and associated description that follows.

#### BRIEF DESCRIPTION OF THE DRAWINGS

FIGS. 1A-1C present schematic representations of semiconductor device cross-sections at various stages of TSV processing.

FIGS. 2A-2C present process flow diagrams illustrating processes for high rate electroplating in accordance with various embodiments.

FIG. 3 is a plot illustrating copper and sulfuric acid concentrations attainable in electrolyte solutions at different temperatures.

FIG. 4 is a plot illustrating solubility of copper salt in electrolyte solutions containing sulfuric acid at 0° C.

FIG. 5 is a computational modeling plot illustrating an increase in plating rates at higher temperatures due to increases in both solubility and in diffusion coefficient of Cu<sup>2+</sup> at higher temperatures.

FIG. 6 is a simplified schematic presentation of an electroplating apparatus equipped with a concentrator module in accordance with an embodiment presented herein.

FIG. 7 is a simplified schematic presentation of an electroplating apparatus adapted for forming a concentrated electrolyte solution in accordance with another embodiment presented herein.

#### DETAILED DESCRIPTION OF A PREFERRED EMBODIMENT

In the following description, the invention is presented in terms of certain specific configurations and processes to help explain how it may be practiced. The invention is not limited to these specific embodiments. Examples of specific embodiments of the invention are illustrated in the accompanying drawings. While the invention will be described in conjunction with these specific embodiments, it will be understood that it is not intended to limit the invention to such specific embodiments. On the contrary, it is intended to cover alternatives, modifications, and equivalents as may be included within the scope and equivalents of the appended claims. In the following description, numerous specific details are set forth in order to provide a thorough understanding of the present invention. The present invention may be practiced without some or all of these specific details. In

other instances, well known process operations have not been described in detail in order not to unnecessarily obscure the present invention.

In this disclosure various terms are used to describe a semiconductor work piece. For example, "wafer" and "substrate" are used interchangeably. The process of depositing, or plating, metal onto a conductive surface via an electrochemical reaction is referred to generally as electroplating or electrofilling. Copper-containing metal in this application is referred to as "copper" which includes without limitation, pure copper metal, copper alloys with other metals, and copper metal impregnated with non-metallic species, such as with organic and inorganic compounds used during electrofill operations (e.g., levelers, accelerators, suppressors, surface-active agents, etc.).

While high rate plating process will be primarily described making reference to copper plating, it is understood that the methods provided herein and associated apparatus configurations can be used to perform high rate plating of other metals and alloys, such as Au, Ag, Ni, Ru, Pd, Sn, Pb/Sn alloy, etc.

Further, while provided methods are particularly advantageous for filling relatively large recessed features, such as TSVs, they can also be used for filling smaller damascene features, or even for high rate plating on planarized substrates.

Electroplating at higher rates is desirable in many areas of semiconductor processing, but is particularly needed for filling relatively large, high aspect ratio recessed features on semiconductor substrates. Specifically, TSVs, which often have a diameter of more than about 3 micrometers and a depth of more than about 20 micrometers, and which in addition can have high aspect ratios (e.g., between about 5:1 and 10:1), are filled relatively slowly when conventional electrolytes and conventional plating systems are used. Further, in conventional systems, filling of such features often results in formation of voids due to disparities in electrodeposition rates at the bottom portions of the features and at the feature openings. For example, if electrodeposition rate at the bottom of the feature is insufficient, while electrodeposition rate at the feature opening is relatively high, the feature opening can close sooner than the feature is fully filled, thereby leaving a void in the feature. Accordingly, while it is generally desirable to increase electrodeposition rates to achieve faster plating, in some embodiments it is also desirable to increase deposition rates at the bottom of recessed feature relative to the deposition rate at the feature opening. In some embodiments, this is achieved by electroplating with electrolytes that have very high Cu<sup>2+</sup> ion concentration at elevated temperatures and with the use of additives which are configured to increase electrodeposition rates at the bottom portion of the recessed feature relative to electrodeposition rates at feature opening.

The highly concentrated electrolytes provided herein typically have component concentrations that exceed their saturation limit at 0° C. The electrolytes are often used at a temperature that is at least about 5 degrees, such as at least about 10 or 20 degrees, higher than the highest temperature at which the electrolyte is fully saturated, to ensure that no precipitation would occur during plating. In this application the "fully saturated electrolyte" refers to the composition that would have normally started to form a precipitate at the temperature to which the reference is made. In other words, concentrated electrolytes provided herein would have formed a precipitate at 0° C. but are typically used at a temperature of at least about 20° C., such as at a temperature of at least about 40° C. (e.g., at a temperature of between

about 40° C. and 75° C.), at which temperatures all electrolyte components remain fully dissolved.

Such concentrated electrolytes typically are not commercially available. For example, when electrolytes containing copper sulfate and sulfuric acid are sold, even most concentrated mixtures, are designed such that they are capable of withstanding shipping and storage temperatures (e.g., 0° C.-10° C.) without forming a precipitate, and therefore have lower concentrations than those desirable for plating in accordance with provided embodiments. Accordingly, methods for preparing concentrated electrolytes prior to plating, and an associated apparatus which includes concentrated electrolyte preparation module, are provided.

In some embodiments, the use of concentrated electrolytes provided herein allows complete filling of a TSV having a diameter of at least about 3 micrometers and a depth of at least about 20 micrometers over a period of less than about 20 minutes and in a substantially void free manner. In some embodiments, electrodeposition rates that are at least 5 times greater than rates obtained using conventional plating conditions are provided. For example plating rates of between about 10,000-50,000 Å/minute as measured based on the filled depth of the via as a function of time, can be achieved. In some embodiments, plating rates of at least about 25,000 Å/minute are preferred.

#### TSV Processing

The integration of provided plating methods into damage feature processing, will be now illustrated making reference to FIGS. 1A-1C, which show cross-sectional views of a substrate containing a through-silicon via (TSV) during various stages of processing.

A TSV is a vertical electrical connection passing completely through a silicon wafer or a die. TSV technology may be used in 3D packages and 3D integrated circuits, sometimes collectively referred to as 3D stacking. For example, a 3D package may contain two or more integrated circuits (ICs) stacked vertically so that they occupy less space and have shorter communication distances between the various devices than in a 2D layout. Traditionally, stacked ICs are wired together along their edges, but such wiring design can still lead to significant signal transmission time delays, as well as to increases in the stack's dimensions, and usually requires additional redistribution layers to route signals to the periphery of the various ICs. Significantly greater numbers of shorter length, dense interconnections can be made by wiring the IC's directly through the silicon substrate, between each of the vertically stacked ICs. TSVs provide connections through the body of the ICs substrate leading to smaller compact stacks with greatly increased communication bandwidth. Similarly, a 3D single IC may be built by stacking several silicon wafers and interconnecting them vertically through each of the substrates. Such stacks behave as a single device and can have shorter critical electrical paths leading to faster operation. This approach is in many aspects technically superior to traditional peripheral wire-bonding interconnect methodology.

Electronic circuits using TSVs may be bonded in several ways. One method is "wafer-to-wafer", where two or more semiconductor wafers having circuitry are aligned, bonded, and diced into 3D ICs. Each wafer may be thinned before or after bonding. The thinning process includes removal of the wafer material to expose the bottom part of the TSV. TSVs may be formed into the wafers either before bonding or created in the stack after bonding and may pass through the silicon substrates between active layers and an external bond pad. Another method is "die-to-wafer" where only one wafer is diced and then the singled dies are aligned and bonded

onto die sites of the second wafer. The third method is "die-to-die" where multiple dies are aligned and bonded. Similar to the first method, thinning and connections may be built at any stage in the last two methods. The integration of the high rate plating process into through-silicon via processing is not significantly affected by the sequence in which the through-silicon via is processed.

FIGS. 1A-1C illustrate processing of a TSV prior to wafer thinning, that is, the TSV at these processing stages does not reach all the way through the silicon wafer. A TSV may be used with both dies and wafers, generally referred here as semiconductor substrate 101. Examples of the material suitable for a semiconductor substrate 101 include, but are not limited to silicon, silicon on insulator, silicon on sapphire, and gallium arsenide. In some embodiments, the semiconductor substrate includes a layer of dielectric, such as silicon oxide based dielectric. In other cases the substrate may be more similar to a single level or multilevel circuit board, and can be made of a ceramic or embedded epoxy. Further in some embodiments the substrate may include circuitry or active transistor devices. These features are not shown to preserve clarity.

In a first cross-sectional view shown in FIG. 1A, a TSV hole 103 is formed in the semiconductor substrate 101. The depth of the TSV hole 103 must be sufficient to allow for a complete cutting through layer 101 during the subsequent thinning operation. Typically, TSV holes may be between about 5 to 400 microns deep (often between about 50 to 150 microns deep), however the present invention may be practiced with the TSV holes of other sizes as well. The diameter of TSV holes may vary between about 1 to 100 microns (more typically between about 5 to 25 microns). The TSV holes typically have a high aspect ratio, which is defined as the ratio of the TSV hole depth to the TSV hole diameter (usually at the opening). In certain embodiments, the TSV hole aspect ratio may vary between about 2:1 to 12:1 (such as between about 3:1 and 10:1). TSV size also depends on which stage of the overall 3D stacking process includes TSV formation. A TSV can be formed before ("via first") or after ("via last") stacking. In the "via-first" configuration, the TSV may be formed before or after creating CMOS structures. In the "via-last" configuration, the TSV may be formed before or after bonding. Moreover, in both configurations, thinning may be performed before or after bonding. The invention may be practiced with any TSV sizes or forming configurations described herein. Table 1 summarizes typical TSV dimensions (in micrometers) for various TSV configurations. While FIGS. 1A-1C and the corresponding description generally pertains to the configuration where a TSV is formed before stacking and CMOS processing and thinning are performed before bonding ("via-first"+ before CMOS+thinning before bonding), this invention can be readily applied to other configurations.

TABLE 1

|    | Via - First |                 |             |            | Via - Last     |               |  |  |
|----|-------------|-----------------|-------------|------------|----------------|---------------|--|--|
|    | Diameter    | Thinning Before | Before CMOS | After CMOS | Before Bonding | After Bonding |  |  |
| 60 | Depth       | Bonding         | 30-50       | 40-150     | 50-400         | 30-150        |  |  |
| 65 | Diameter    | Thinning After  | 1-5         | 1-5        | 3-5            | 3-5           |  |  |
|    | Depth       | Bonding         | 5-25        | 5-25       | 5-25           | 5-25          |  |  |

TSV holes may be formed using standard photolithographic and etching methods. Returning to FIG. 1A, the

TSV hole 103 may be formed through a top surface, which may be an active surface of a wafer or a die and may include electronic devices. Alternatively, the TSV hole may be formed through the back surface of a wafer or a die where the circuitry is not present.

The cross-section in FIG. 1A shows that a layer of diffusion barrier material 105 resides over the substrate 101, and conformally lines the substrate both in the field and within the TSV 103. Suitable materials for the diffusion barrier layer 105 include tantalum, tantalum nitride, tungsten, titanium, ruthenium, titanium nitride, and alloyed and layered combinations of these and other materials. In a typical embodiment, the diffusion barrier layer 105 is formed by a PVD process, although other techniques such as chemical vapor deposition (CVD), electroless deposition, or atomic layer deposition (ALD) may be employed. The seed layer 107 is then deposited to provide a uniform conductive surface for current passage during an electroplating operation. As with the barrier layer deposition, a PVD method may be employed for this operation, although other processes such as electroless or electrolytic deposition may be employed as well. Suitable seed layer materials include metals such as copper, copper alloys, cobalt, nickel, ruthenium, etc. or combined layers such as Co/Cu or Ru/Cu. In some embodiments the seed layer can also perform a function of a diffusion barrier. In these embodiments, it may not be necessary to employ a separate diffusion barrier layer 105. Referring again to FIG. 1A, it can be seen that seed layer 107 conformally lines the substrate and resides on top of the diffusion barrier layer 105 both in the field and within the TSV.

Next, a copper layer 111 is deposited by electroplating onto the seed layer 107 (the seed layer is not shown in FIG. 1B to preserve clarity) to completely fill the TSV hole 111, as shown in FIG. 1B. Concentrated electrolyte solutions containing very high Cu<sup>2+</sup> concentrations are used in the plating process, preferably at elevated temperature of at least about 40° C. Electrolyte chemistry and plating conditions will be described in detail in the subsequent sections. During plating current is generated through the seed layer 103 causing copper ions to flow towards and deposit on the seed layer. Typically, during electrodeposition a copper overburden layer 109 is formed over the field region. In large feature size 3D packaging (e.g. TSV) application overburden typically has a thickness ranging from about 4 micrometers to 25 micrometers. In some embodiments, little or no overburden may form on the substrate after the TSV is filled. Suitable electrolyte chemistry for plating with little or no overburden is described in the commonly owned U.S. patent application Ser. No. 12/193,644, filed on Aug. 18, 2008, titled "Process for Through Silicon Via Filling" naming J. Reid et al. as inventors, which is herein incorporated by reference in its entirety.

After electrodeposition of copper is completed, the overburden 109 is removed in a post electroplating process, which may include wet chemical etching, chemical mechanical polishing (CMP), electroplanarization, and various combinations of these methods.

The next cross-section shown in FIG. 1C illustrates the substrate 101 after post-electroplating processes to remove copper overburden are completed. As shown, the overburden 109 is removed and the diffusion barrier layer 105 is exposed over the field region. In subsequent operations (not shown), the diffusion barrier material is removed from the field region (e.g., by CMP) and the substrate is thinned at the TSV bottom, to allow the TSV go entirely through the substrate. Electrolyte Chemistry and Electrolyte Preparation

An exemplary method for high rate electroplating is illustrated in the process flow diagram shown in FIG. 2A. In 201 a semiconductor substrate having a recessed feature is received. For example, the substrate may be a wafer or a die having one or more TSV holes. Independently, in operation 203, a highly concentrated electrolyte solution is prepared. The highly concentrated electrolyte has Cu<sup>2+</sup> concentration in excess of saturation limit at 0° C. The prepared electrolyte is maintained at a temperature that is at least about 10° C. higher than the highest temperature at which the solution is fully saturated (i.e. the highest temperature at which precipitate would have formed). For example, in some embodiments, the concentrated electrolyte is fully saturated at 0° C. and is maintained at room temperature (about 20° C.). In other embodiments, the concentrated electrolyte is fully saturated at room temperature (at 20° C.) and is maintained at a temperature of at least about 40° C., such as at a temperature of between about 40-75° C., for example at a temperature of between about 50-70° C.

The prepared electrolyte solution contains one or more copper salts, which may include without limitation copper sulfate, copper methanesulfonate, copper propanesulfonate, copper gluconate, copper pyrophosphate, copper sulfamate, copper nitrate, copper phosphate, copper chloride, and their various combinations.

In some embodiments, the prepared concentrated electrolyte further includes an acid, such as sulfuric acid, methanesulfonic acid, propanesulfonic acid, nitric acid, phosphoric acid, hydrochloric acid and various combinations thereof. For example, the electrolyte solution in one embodiment contains copper sulfate and sulfuric acid.

In some embodiments, although not necessarily, the concentrated solution provided herein has a relatively high concentration of acid in addition to high concentration of Cu<sup>2+</sup>. This is particularly significant for TSV filling because a voltage drop in the electrolyte solution within the via results in a reduced plating rate at the base of the via relative to the field region. This voltage drop can be reduced by using an electrolyte having a relatively high acid concentration. For example, in some embodiments, the concentrated electrolyte solution contains an acid at a concentration of between about 0.1-2 M, such as between 0.4-2 M, e.g., between about 1-2M. In some embodiments, solutions with acid concentration of at least about 0.6 M are used. For example, sulfuric acid is used in some embodiments at a concentration range of between about 40 and 200 g/L, preferably at a concentration of at least about 60 g/L. For example, the concentrated electrolyte solution may contain Cu<sup>2+</sup> and H<sub>2</sub>SO<sub>4</sub>, where the solution is fully saturated at 0° C., or, in some embodiments, is fully saturated at 20° C., where the concentration of H<sub>2</sub>SO<sub>4</sub> is relatively high, such as between about 100 and 200 g/L. Such concentrated solutions, are prepared in some embodiments by concentrating a solution containing Cu<sup>2+</sup> and one or more acids (e.g., H<sub>2</sub>SO<sub>4</sub>, an alk), where the volume of solution is reduced between about 1.5-3 fold. In other embodiments, such solutions are prepared by mixing acid solution with a solution containing Cu<sup>2+</sup>.

The actual concentration of copper ion that can be achieved in the provided concentrated electrolyte will depend on selected operating temperatures and on the presence of other components, such as an acid having common anion. As the solubility of copper salts increases with increasing temperature, significantly higher concentrations of Cu<sup>2+</sup> cation can be achieved by maintaining and using the highly concentrated electrolyte at higher temperatures.

## 11

The solubility of a particular salt is given by its solubility product,  $K_{sp}$ . The salt precipitates after its solubility product value for a give temperature is reached. For example, for copper sulfate the solubility product is the product of copper ion and sulfate ion molar concentrations:

$$K_{sp} = [Cu^{2+}][SO_4^{2-}]$$

For those electrolyte solutions which contain both copper sulfate and sulfuric acid, the increase in sulfuric acid concentration increases sulfate ion concentration and thereby causes precipitation of copper sulfate at a lower  $Cu^{2+}$  concentration (compared to pure copper sulfate solution). This is illustrated, for example by a plot shown in FIG. 3, which shows  $Cu^{2+}$  concentration (in g/L) and  $H_2SO_4$  concentration (in g/L) at which solubility product is reached at 0° C. ( $K_{sp1}$ ) and at about 20° C. ( $K_{sp2}$ ). It can be seen that when acid concentration is 0, the solubility product is reached at 0° C. at  $Cu^{2+}$  concentration of about 80 g/L. When the concentration of sulfuric acid is increased to about 120 g/L, the solubility product is reached at about 30° C. at lower  $Cu^{2+}$  concentration of about 40 g/L.

Therefore, the concentration of  $Cu^{2+}$  in provided highly concentrated electrolytes can differ in different embodiments depending on the operating temperatures and composition of solution. In some embodiments, the concentration of  $Cu^{2+}$  is at least about 40 g/L, such as at least about 60 g/L, for example at least about 80 g/L, such as between about 100-200 g/L.

In some embodiments, the concentrated electrolyte contains at least one copper salt, for which the solubility product at 0° C. is exceeded, for example, by at least 5, 10, 20, or 50%, while the concentrated electrolyte is maintained at a temperature of at least about 20° C. In some embodiments, the concentrated electrolyte contains at least one copper salt, for which the solubility product at 20° C. is exceeded, for example, by at least 5, 10, 20, or 50%, while the concentrated electrolyte is maintained at a temperature of at least about 40° C.

Exemplary suitable concentrated solutions are illustrated in the plot shown in FIG. 4, which illustrates saturation of  $CuSO_4$  in the presence of sulfuric acid at 0° C. The marked area above the line illustrates the concentrations of  $Cu^{2+}$  in g/L and  $H_2SO_4$  in g/L which correspond to complete saturation at 0° C. For example, an electrolyte solution containing 80 g/L  $Cu^{2+}$ , 10 g/L  $H_2SO_4$ , and 50 mg/L  $Cl^-$  represented by the black dot will be beyond saturation limit at 0° C., while a solution containing 70 g/L  $Cu^{2+}$ , 10 g/L  $H_2SO_4$ , and 50 mg/L  $Cl^-$  will not exceed solubility product at this temperature.

In one example, the concentrated electrolyte solution contains copper sulfate and sulfuric acid, with  $Cu^{2+}$  concentration of between about 60-120 g/L and  $H_2SO_4$  concentration of between about 5-75 g/L. In some embodiments, provided electrolytes have the chemistry described in U.S. patent application Ser. No. 12/193,644, which was previously incorporated by reference.

Thus, the concentrated electrolyte solutions may contain one or more copper salts, and, optionally, an acid. The concentrated electrolyte solutions may be prepared in a number of ways. In one embodiment, the concentrated electrolyte solution is prepared from a less concentrated solution (also referred to as a non-concentrated solution) by removing water, such as by evaporation or reverse osmosis. In another embodiment the concentrated solution is prepared by combining a relatively concentrated solution containing copper salt with a solution of acid to form a solution that exceeds its saturation limit at 0° C. The formed solution is

## 12

maintained at a temperature of at least about 20° C. In other embodiments, a combination of these methods may be used. For example, a relatively concentrated copper salt solution (e.g., having  $Cu^{2+}$  concentration of greater than 65 g/L) can be combined with a concentrated or non-concentrated acid solution, and the resulting mixture may be concentrated, e.g., by evaporation or reverse osmosis, to achieve an even greater concentration of cupric ion (e.g., greater than 85 g/L). The formed solution may be maintained at room temperature, or elevated temperature depending on the level of concentration.

Referring again to the process shown in FIG. 2A, after the concentrated solution has been prepared, or concurrently with the preparation of concentrated electrolyte solution, one or more additives may be optionally introduced to the plating solution in operation 205. The additives typically include one or more of levelers, accelerators, suppressors, and surface-active agents, and are configured to increase electroplating rates at the recessed feature bottom relative to the plating rates in the field region, or, in other words, to suppress plating on the wafer field relative to the recessed feature bottom.

Accelerators may include a sulfur, oxygen, or nitrogen functional group that help to increase deposition rates and may promote dense nucleation leading to films with a fine grain structure. Accelerators may be present at a low concentration level, for example 0-200 ppm. While the accelerator may produce high deposition rates within the TSV hole, the accelerator may be transported away from the substrate top surface (field region) and/or consumed by reaction with oxygen in the bulk solution. Suppressors are additives that reduce the plating rate and are usually present in the plating bath at higher concentrations, for example 5-1,000 ppm. They are generally polymeric surfactants with high molecular weight, such as polyethylene glycol (PEG). The suppressor molecules slow down the deposition rate by adsorbing on the surface and forming a barrier layer to the copper ions. Because of their large size and low diffusion rate, suppressors are less likely to reach the lower part of the TSV than the wafer field resulting in lower concentrations at the bottom of the TSV. Therefore, most of suppressing effect occurs on the surface of the substrate (field region), helping to reduce overburden and avoid TSV hole "closing". Levelers are the additives whose purpose is to reduce surface roughness. They are present, if at all, in very small concentrations, such as 1-100 ppm, and their blocking effects at the surface are highly localized. As a result, levelers selectively reduce deposition mainly on the high spots allowing the low spots to level out. This behavior can also be used to enhance the plating rate of copper at the base of the TSV relative to the growth rate on the wafer field. In some cases, levelers may contain functional groups which include nitrogen atoms which exhibit a tendency to form complexes with  $Cu(I)$  ions at the wafer interface. Finally, chloride ions may be present in the plating bath at a concentration of no greater than about 300 ppm.

In some embodiments, the additives reduce the current density (and the plating rate) in the field and at the upper lip of the TSV twofold relative to the current density in the field that would have been obtained in the absence of additives. The additives help achieve void-free filling by increasing the relative plating rate at feature bottom relative to feature opening. The additives can operate in synergy with high concentration of  $Cu^{2+}$  and high temperature conditions to achieve the goal of void-free filling, which is particularly important for high aspect ratio TSV filling.

After the electrolyte has been formed, in operation 207, the substrate is contacted with the highly concentrated electrolyte solution to at least partially fill the recessed feature. The temperature in the plating cell is controlled such that the precipitation of electrolyte is avoided. For example, if the electrolyte is saturated at 0° C. (as highest saturation temperature) then plating can be performed at 20° C. or higher. If the highest temperature at which the electrolyte is saturated is 20° C., the temperature in the plating bath can be maintained at 40° C. and higher. In some embodiments, plating is performed at a temperature of at least about 50° C., such as at a temperature of about 60° C.

The electrolyte can be provided to the plating cell continuously, semi-continuously, or incrementally. Optionally, as depicted in operation 209, the highly concentrated electrolyte solution is recirculated, for example by continuously or incrementally removing the highly concentrated electrolyte from an electrolyte exit port in the plating cell, passing it through a filter and optionally through a degasser and eventually returning it back to the plating cell. Care is taken to control the temperature of the concentrated electrolyte during recirculation in order to avoid inadvertent precipitation of copper salt.

FIGS. 2B and 2C are illustrative examples of process flows which involve different methods of preparing concentrated electrolyte for plating. The process shown in FIG. 2B starts in 211 by receiving a non-concentrated electrolyte containing  $\text{Cu}^{2+}$  ion. For example, the electrolyte can be an aqueous solution of copper salt, which optionally may include an acid. In some embodiments, the received non-concentrated electrolyte is a solution consisting essentially of copper salt (e.g., copper sulfate), an acid (e.g. sulfuric acid), and, optionally, a halide (e.g., chloride). In some embodiments, the non-concentrated solution may also include one or more organic additives. The concentration of  $\text{Cu}^{2+}$  ion in the non-concentrated solution is such that the solution is not fully saturated at 20° C.—that is the concentrations of components are below the concentrations that would have resulted in precipitation. For example, the non-concentrated solution can comprise a copper salt at less than about 90% of its  $K_{sp}$  at 20° C., such as at less than about 80% of  $K_{sp}$  at 20° C., or even less than about 50% of its  $K_{sp}$  at 20° C. Non-concentrated solutions can be obtained commercially. For example a solution containing 40 g/L  $\text{Cu}^{2+}$  and 10 g/L  $\text{H}_2\text{SO}_4$  can be commercially obtained from ATMI, Danbury, Conn.

In operation 213 the non-concentrated electrolyte is concentrated to obtain a highly concentrated electrolyte solution. The obtained solution is maintained at a temperature of at least about 40° C. The formed highly concentrated solution would have been fully saturated (i.e. would have formed a precipitate) at 20° C., but is maintained at a temperature of at least about 40° C. (e.g., at a temperature of at least about 50° C.) such that copper salt or salts remain fully dissolved. The concentration can be performed in a concentrator module configured for removing water from non-concentrated solution and for controlling and maintaining required temperatures and concentrations in the prepared electrolyte solution. In some embodiments, the volume of solution is reduced about 1.5-3 fold. In some embodiments, water is removed by evaporation of water, which may be performed in a temperature range of between about 40-100° C., preferably at between about 80-100° C. In some embodiments the solution is brought to boiling and water is removed while the solution is boiled. Dry air may be introduced into the concentrated air module through a dry air port, and wet air may be removed through a wet air port to facilitate the

concentration process. This type of concentrator module will be described in additional detail in the “Apparatus” section.

In other embodiments, the water is removed in the concentrator module by reverse osmosis. In these embodiments, the concentrator module will typically include a chamber or a line for providing the non-concentrated electrolyte solution, a semipermeable membrane connected with this chamber or line, and a chamber or a line configured for holding or discarding removed water. A high-pressure pump is included in the system, which exerts the required pressure on the electrolyte solution such that water passes through the semipermeable membrane, thereby concentrating the electrolyte. Once the electrolyte is sufficiently concentrated, care is taken to maintain it at a temperature of at least about 40° C. to avoid precipitation. The reverse osmosis concentrator may include one or more heaters, concentration detectors, and temperature detectors electrically connected with one or more controllers configured for controlling and maintaining concentrations and temperatures.

20 After the highly concentrated electrolyte has been prepared in the concentrator module, it is directed from an outlet port in the concentrator module to a concentrated electrolyte reservoir. As stated in operation 205, the concentrated electrolyte reservoir is configured to maintain the 25 concentrated solution at a temperature of at least about 40° C. to avoid salt precipitation from the highly concentrated electrolyte. The concentrated electrolyte reservoir includes a vessel configured for holding the concentrated electrolyte. The reservoir typically includes a heater and a temperature 30 sensor connected to a controller, which is configured to maintain the electrolyte at a desired temperature. The reservoir may also include a concentration sensor (e.g., an optical sensor configured for measuring optical density of the electrolyte solution) connected with a concentration controller. The temperature of the electrolyte in the reservoir 35 need not necessarily be the same as the temperature of the electrolyte in the concentrator. While it is important that both in the concentrator and in the reservoir the temperature is maintained above the temperature at which precipitation occurs, these temperatures need not be identical. For 40 example, in some embodiments, the water may be removed in the concentrator at a temperature of at least about 80° C., while the electrolyte may be maintained in the reservoir at lower temperatures of between about 40-65° C. Further, the composition of the concentrated electrolyte in the concentrator and in the reservoir need not necessarily be identical. For 45 example, in some embodiments, the electrolyte in the reservoir may include organic additives, while the electrolyte in the concentrator may be additive-free, in order to minimize exposure of organic additives to high temperatures in the concentrator. In other embodiments, the concentrated electrolyte in the concentrator does not include an acid, and the acid is added to the electrolyte in the reservoir. Also, in 50 some embodiments, the electrolyte in the concentrator may be more concentrated than the electrolyte in the reservoir (while both are highly concentrated and exceed saturation limit at 20° C.).

As shown in operation, 217 one or more additives may 55 optionally be added to the electrolyte in the reservoir. The additives may include one or more of accelerators, suppressors and levelers, as previously described.

Next, in operation 219 the concentrated electrolyte is directed to the plating cell where it is contacted with the substrate to deposit copper at a temperature of at least about 40° C. (e.g., at a temperature of between about 40-80° C., such as at between about 50-75° C.). The temperature in the plating cell need not be necessarily the same as in the

reservoir or in the concentrator but should be sufficient to keep the copper salts from precipitating from the electrolyte solution. The plating cell may include an electrolyte concentration sensor connected with the electrolyte concentration controller. In some embodiments the plating cell does not include a heater, and the warm concentrated electrolyte is supplied from the reservoir continuously or semi-continuously without allowing significant cooling of the electrolyte in the cell. In other embodiments, the plating cell may include a heater connected to a temperature controller. The described embodiment provides an integrated system for forming a highly concentrated electrolyte from commercially available non-concentrated electrolyte and for maintaining the electrolyte at an elevated temperature during preparation in the concentrator module, storage in the reservoir, and use in the plating cell.

Another embodiment involving preparation of highly concentrated electrolyte solution is shown in FIG. 2C. This method starts in operation 221 by receiving a solution of copper salt and a solution of an acid. For example a concentrated solution of copper sulfate having  $Cu^{2+}$  concentration of between about 65-85 g/L is provided. Such concentrated solution can be purchased, e.g., from ATMI, Danbury, Conn. or prepared by dissolution of solid copper sulfate in water. In some embodiments copper sulfate solution having this or even higher concentration is prepared by dissolution of solid copper sulfate in water at an elevated temperature.

Further, a concentrated solution of sulfuric acid (e.g., 900-1800 g/L  $H_2SO_4$ ) is provided. Concentrated sulfuric acid is readily commercially available. Next, in operation 223, the solution of copper salt is combined with the solution of the acid in a reservoir to form a concentrated electrolyte solution. In some embodiments, the resulting concentrated electrolyte solution exceeds its saturation limit (would have formed a precipitate) at 0° C., and the resulting solution is maintained at a temperature of at least about 20° C., e.g., at about 20-35° C. In other embodiments, the resulting highly concentrated solution exceeds its saturation limit at 20° C. and is maintained at a temperature of at least about 40° C.

The concentrated copper salt solution and the concentrated acid solution can be mixed in a reservoir, which may, depending on the embodiment, include a heater and a temperature controller. In some embodiments, the heat generated by mixing these components is utilized, and no additional heater may be required. In some embodiments the components are mixed in delivery lines without having a dedicated reservoir for holding the resulting highly concentrated solution.

In operation 225, one or more additives, such as accelerators, suppressors, levelers and their various combinations are optionally added to the highly concentrated electrolyte solution.

In operation 227, the solution is directed to the plating cell where the concentrated electrolyte contacts the substrate to deposit copper at a temperature that is sufficient for the concentrated electrolyte to be fully in solution. In some embodiments, the temperature during plating is between about 20-35° C. In other embodiments it is preferable to plate at a temperature of at least about 40° C., such as at a temperature of between about 40-65° C.

#### Effect of High Copper Concentration and High Temperature on Deposition Rates

During electroplating on substrates containing TSVs the maximum current of operation (and electroplating rate) is limited by the depletion of  $Cu^{2+}$  ion near the base of the vias. This depletion is described in detail in the U.S. application

Ser. No. 12/193,644 which was previously incorporated by reference. By increasing the concentration of  $Cu^{2+}$  in electrolyte solution, preferably in combination with increase in temperature of the electrolyte the current at the via base can be significantly increased. The increase in current and associated increase in the plating rate is both due to higher diffusion coefficient of copper at higher temperature and due to the greater concentration of  $Cu^{2+}$  ions in the bulk solution that can be achieved at higher temperature. The actual observed plating rate correlates with the product of these two parameters, and, therefore, unexpectedly high rates of plating can be achieved with highly concentrated electrolytes at elevated temperatures. FIG. 5 illustrates how relative diffusion coefficient (diamond-marked curve), relative copper solubility (square-marked curve), and their product (triangle-marked curve) increase with increasing temperature. All parameters are related to corresponding parameters at 20° C. Thus, all three parameters at 20° C. have the value of 1. When temperature is increased from 20° C. to 60° C., the relative solubility of copper sulfate increases to about 2, while  $Cu^{2+}$  diffusion coefficient increases to about 2.5. The plating rate which correlates with the product of these values, will, accordingly be increased to about 5, relative to the plating rate observed at 0° C.

FIG. 5 illustrates how the maximum plating rate varies as a function of temperature due to both the effect of increased copper solubility and increased diffusion coefficient. It is seen that diffusion and solubility effects taken separately, have a similar degree of benefit as a function of temperature, and that the combined benefit is a product of the individual effects. As a result, the relative diffusion limited current becomes very large when high temperature plating is used in combination with the use of highly concentrated electrolytes that can be attained at high temperatures. This effect of sharply higher capability to deliver  $Cu^{2+}$  ion to the plated interface due to the combination in increase in diffusion coefficient and copper bulk concentration allows for more rapid  $Cu^{2+}$  ion replenishment in the TSV bottoms at a given current setting.

Table 2 lists computer modeling results illustrating concentration, voltage, and current profile behavior in TSVs as a function of higher copper concentration and increased temperature. The modeling shows that nearly a six-fold increase in plating rate (and TSV base current) can be achieved while maintaining a constant degree of cupric ion depletion near the feature base when the copper concentration is increased from 60 to 120 g/L and the bath temperature is increased from 20 to 65° C.

TABLE 2

|                                      | Field current          | Via base current       | Voltage drop in via | Cu depletion at via base |
|--------------------------------------|------------------------|------------------------|---------------------|--------------------------|
| Case 1: 20 C. 60 g/L Cu 10 g/L Acid  | 3.6 mA/cm <sup>2</sup> | 1.6 mA/cm <sup>2</sup> | 3.8 mV              | 35%                      |
| Case 2: 65 C. 60 g/L Cu 10 g/L Acid  | 12 mA/cm <sup>2</sup>  | 5.3 mA/cm <sup>2</sup> | 5.2 mV              | 39%                      |
| Case 3: 65 C. 120 g/L Cu 20 g/L Acid | 22 mA/cm <sup>2</sup>  | 9.6 mA/cm <sup>2</sup> | 4.9 mV              | 36%                      |

#### Apparatus

The apparatus for practicing described methods typically includes one or more plating cells and one or more modules for preparing concentrated electrolyte solution, where the modules are configured for providing concentrated electrolyte into the plating cells. The apparatus also includes a

controller, which controls electrolyte concentrations and temperatures during various stages of electrolyte preparation and use, and is configured to prevent precipitation of copper salts during electrolyte preparation and use. In some embodiments the apparatus includes a reservoir configured for holding the concentrated electrolyte (e.g., during or after preparation) and delivering it to the plating cell. In some embodiments, the reservoir is configured for preparing and/or storing concentrated electrolyte solution at a volume that is between about 10-50% greater than the volume of electrolyte in the plating cell during use.

FIGS. 6 and 7 provide simplified schematic presentations of two different types of apparatus in accordance with the embodiments provided herein. It is understood that these are exemplary configurations, and that various modifications of these configurations are possible, as will be appreciated by one of skill in the art.

FIG. 6 illustrates an apparatus having a concentrator module 601, a reservoir 603, and a plating cell 605. This apparatus is suitable for practicing the plating method illustrated by the process flow diagram shown in FIG. 2B. In the configuration presented in FIG. 6, the non-concentrated electrolyte is concentrated in the concentrator module 601 by high-temperature evaporation. The non-concentrated electrolyte is provided from the source of non-concentrated electrolyte 609, which may be a tank configured for holding non-concentrated copper salt, and, optionally, an acid. In one embodiment source 609 holds copper sulfate and sulfuric acid at such concentrations that the solution is not saturated at 0° C. The non-concentrated electrolyte solution is delivered through the non-concentrated electrolyte entry port 635 into the concentrator 601. The delivery of the non-concentrated solution is controlled by a valve 637. The non-concentrated electrolyte may be a copper salt solution which may optionally include an acid. In other embodiments the concentrator receives copper salt from a source of a copper salt, and, separately, an acid from a source of an acid, and the components are mixed within the concentrator.

The concentrator is equipped with a heater 615 a temperature sensor (not shown) and an optical concentration sensor 639, which are connected to the controlling unit 625 (only one connection 645 is shown to preserve clarity). The concentrator is further has an inlet port 630 adapted for receiving a diluent, such as deionized water from a diluent source 651. The flow of diluent is controlled by valves 627 and 629, of which valve 629 is connected with an overflow shutoff member 651 configured to close valve 629 if overflow is detected in the concentrator module. The concentrator also includes an emergency overflow conduit 643, which is configured to remove excess electrolyte if the electrolyte level exceeds a threshold value. In some embodiments the overflow concentrated electrolyte is diluted in the overflow conduit 643 or afterwards to prevent precipitation of copper salts upon cooling of overflow. The concentrator 601 further includes a recirculation loop for recirculating concentrated electrolyte and for directing the concentrated electrolyte to the concentrated electrolyte reservoir. The concentrator includes an outlet port 641 through which the concentrated electrolyte exits the concentrator vessel. The concentrated electrolyte is pumped with the use of pump 617 through filter 647 and is optionally passed through a degasser (not shown) and is returned to the concentrator vessel through entry port 649. The concentrated electrolyte can be diverted from the recirculation loop at junction 653 and can be directed to the concentrated electrolyte reservoir 603, which it enters at the concentrated electrolyte entry port 663. The flow of concentrated electrolyte to the concentrated electro-

lyte reservoir is controlled by valve 654. The concentrator module 601 in the illustrated embodiment is configured to heat the electrolyte to a temperature of at least about 40° C., such as to at least about 80° C. and to remove water by evaporation. To facilitate evaporation of water the concentrator vessel includes an entry port 631 configured for receiving dry air and an exit port 633 configured for removing wet air. It is understood that a variety of alternative ways to facilitate removal of water in the concentrator may be used. For example in some embodiments, water may be removed under reduced pressure. The concentrator is configured to produce a highly concentrated electrolyte that would have been fully saturated at 0° C., and, in some embodiments, an electrolyte that would have been fully saturated at 20° C. In some embodiments the concentrator reduces the volume of received non-concentrated electrolyte by at least 1.5 times, such as by between about 1.5-3 times. In other embodiments the concentrator module is adapted for removing water by other methods, such as by reverse osmosis. A concentrator adapted for reverse osmosis has been previously described with reference to FIG. 2B.

After the concentrated electrolyte solution exits the concentrator recirculation loop at 653 it is directed to the concentrated electrolyte reservoir 603 through port 663. The concentrated electrolyte reservoir is configured for holding the concentrated solution and for delivering it to the plating cell 605. The reservoir in this configuration is equipped with an immersion heating element 619 and a temperature sensor and is configured for maintaining the electrolyte at a temperature of at least about 40° C., such as at about 40-80° C., e.g., at between about 40-65° C., or at about 50-65° C. The reservoir may also include one or more concentration sensors. Any of the temperature and concentration sensors as well as the heating element may be electrically connected through connection 655 to the controller unit 625 which is configured to control temperature and concentration of electrolyte in the reservoir in order to maintain the desired high concentration and to keep the copper salts from precipitating in the reservoir. Similarly to the concentrator, the reservoir 603 includes an inlet port 665 configured for addition of diluent, such as deionized water. The diluent is supplied from the diluent source 611, with the flow of diluent being controlled by valves 669 and 667. The valve 667 is connected with the overflow shut-off member 661, which closes the valve 667, when the level of electrolyte in the reservoir reaches a threshold value. The reservoir also includes an emergency electrolyte overflow conduit, which operates similarly to the conduit 643 in the concentrator module. Further, in the provided configuration, the reservoir has an inlet 673 which is configured for receiving electrolyte additives (such as one or more of levelers, accelerators and suppressors), which are delivered from the additive source 613 and are controlled by a valve 671.

In the described configuration the reservoir is adapted for providing the concentrated electrolyte to the plating cell 605 in a continuous or semi-continuous manner. The concentrated electrolyte (which in this embodiment contains copper salt, acid, and additives) is directed through outlet port 679, pump 621, filter 681, and optionally, a degasser to the inlet port 683 of the plating cell. Because the warm electrolyte solution from the reservoir is pumped into the plating cell continuously or semi-continuously, in the depicted configuration it is not necessary to include a heater element in the plating cell. In some embodiments it is possible to maintain the temperature of the electrolyte in the plating cell within about 5° C., such as within about 3° C. of the electrolyte temperature in the reservoir by continuous or semi-continu-

ous pumping. In other embodiments, a heater may be included within the plating cell. The plating cell 605 includes a vessel adapted for holding the electrolyte, a wafer holder (not shown) which is adapted to hold wafer 659 and a motor adapted for rotating the wafer. Within the vessel an anode 623 is disposed typically opposite the wafer 659. The wafer (the cathode) and the anode are electrically connected to a power supply, which provides an appropriate current to the wafer, biasing it negatively versus the anode. As it was previously mentioned, the wafer includes a conductive seed layer on its surface, to which electrical connections are made typically at the periphery of the wafer. During plating, the copper ions in the electrolyte move towards the wafer are reduced at the wafer surface forming the electrodeposited copper layer. The provided depiction of the copper plating cell 605 is simplified to preserve clarity. It is understood that the plating cell may include multiple additional elements. For example, in some embodiments, the plating cell may include an ionically resistive ionically permeable member, such as an insulating plate having multiple non-interconnecting holes, which is disposed in close proximity of the wafer to improve plating uniformity. Further, in some embodiments, the anode in the plating cell may include several segments, which may be surrounded by focusing walls adapted to focus and shape current within the plating cell. Further, the plating cell may include a second cathode (a negatively biased conductive member) adapted to divert current from the edge of the wafer. Further, in some embodiments the anode may be separated from the cathode by an ionically permeable membrane thereby creating separate anode and cathode chambers within the plating cell. It is understood that a variety of different plating cell configurations may be used in conjunction with concentrated electrolyte preparation module described herein.

In the described configuration the electrolyte in the plating cell is recirculated back to the reservoir 603 simply by overflow from the plating cell. In other embodiments, the recirculation loop may include overflow of electrolyte from the reservoir 603 into the plating cell 605 and subsequent direction of used electrolyte back to the reservoir 603 through an exit port, and an exit line equipped with a pump and a filter. In an alternative embodiment, which is not depicted, electrolyte from the plating cell 605 is directed to the concentrator module 601, e.g., by overflow from the plating cell or by a separate line (typically equipped with a pump, filter, and a valve) connecting the plating cell and the concentrator. The electrolyte is then recirculated back to the plating cell from the concentrator through the reservoir.

In some embodiments, the concentrated electrolyte leaving the plating cell 605 is diluted to a concentration at which the electrolyte is stable at 20° C. and is directed to one or more vessels for storage, e.g., during tool idle time. In some embodiments, the diluted electrolyte is directed to the source of non-concentrated electrolyte 609, which is in fluidic communication with the concentrator.

The plating cell may also include one or more temperature and concentration detectors connected through electrical connection 657 to the controller unit 625.

The controller unit 625 may be manually controlled or may include a set of program instructions. The controller may control all or some aspects of electrolyte concentration process, electrolyte storage in the reservoir, and plating. Specifically the controller is adapted to control concentration and temperature in at least one of the concentrator module, the concentrated electrolyte reservoir, and the plating cell, such that desired concentrations are achieved and such that precipitation of copper salts is avoided.

The controller will typically include one or more memory devices and one or more processors. The processor may include a CPU or computer, analog and/or digital input/output connections, stepper motor controller boards, etc.

5 In certain embodiments, the controller controls all of the activities of the electroplating apparatus. The system controller executes system control software including sets of instructions for controlling one or more of temperature in the concentrator, reservoir, or the plating cell, flow of non-concentrated electrolyte into the concentrator, flow of the diluent into the concentrator, flow of the concentrated electrolyte into the reservoir, flow of the diluent into the reservoir, flow of the concentrated electrolyte into the plating cell and other parameters of a particular process. For example, 10 the controller may be adapted to raise the temperature and/or to add the diluent if the electrolyte in the concentrator or reservoir becomes too concentrated or precipitates. The controller may further include instructions for controlling the flow rate from the reservoir to the plating cell, such that 15 the electrolyte does not cool down significantly within the plating cell.

Other computer programs stored on memory devices associated with the controller may be employed in some embodiments.

20 25 Typically there will be a user interface associated with controller 625. The user interface may include a display screen, graphical software displays of the apparatus and/or process conditions, and user input devices such as pointing devices, keyboards, touch screens, microphones, etc.

30 The computer program code for controlling the deposition and resputtering processes can be written in any conventional computer readable programming language: for example, assembly language, C, C++, Pascal, Fortran or others. Compiled object code or script is executed by the processor to perform the tasks identified in the program.

35 The controller parameters relate to process conditions such as, for example, non-concentrated electrolyte composition and flow rates, temperature, additive solution flow rates, etc. These parameters are provided to the user in the form of a recipe, and may be entered utilizing the user interface.

40 45 Signals for monitoring the process may be provided by analog and/or digital input connections of the system controller. The signals for controlling the process are output on the analog and digital output connections of the deposition apparatus.

The system software may be designed or configured in many different ways. For example, various apparatus component subroutines or control objects may be written to control operation of the chamber components necessary to carry out the inventive deposition processes. Examples of programs or sections of programs for this purpose include temperature control code, concentration control code, etc.

50 55 Examples of sensors that may be monitored by the controller during electrolyte preparation and plating include optical concentration detectors, mass flow controllers, density meters, and temperature sensors in the concentrator module, reservoir, or the plating cell. Further, level of electrolyte in the concentrator, reservoir, and the plating cell can be monitored. Appropriately programmed feedback and control algorithms may be used with data from these sensors to maintain desired process conditions. For example, in some embodiments, the controller is configured for rapidly diluting electrolyte and containing the added volume in the concentrator, reservoir, or plating cell, upon drop in temperature or inadvertent concentration increase to prevent precipitate formation. For example, the controller may be

programmed to add water to a predetermined level in one or more of these vessels upon non-planned shut-off of the system, e.g., in response to high concentration or low temperature reading. The system is also equipped with cut-off valves to prevent overflow, which can stop the flow of diluent after the electrolyte reaches a desired level.

In some embodiments the controller includes program instructions to perform the method described with reference to FIG. 2B.

#### Example

In one illustrative example, a non-concentrated electrolyte solution containing copper sulfate and sulfuric acid at a concentration of 60 g/L  $\text{Cu}^{2+}$  and 20 g/L  $\text{H}_2\text{SO}_4$  is added from the tank 609 to the concentrator 601. In the concentrator, the electrolyte is evaporated to 50% of its volume resulting in an electrolyte having a concentration of 120 g/L  $\text{Cu}^{2+}$  and 40 g/L  $\text{H}_2\text{SO}_4$ . The electrolyte is then directed to the reservoir 603, and subsequently to the plating cell 605, while temperature of the electrolyte is always maintained at about 60° C. and above. The plating of copper on the substrate is performed at 60° C. In this case the improvement in plating rate relative to the room temperature bath having 60 g/L  $\text{Cu}^{2+}$  concentration is about 5-fold, which is the product of 2.5-fold increase due to increase in diffusion coefficient at high temperature, and 2-fold increase due to cupric ion concentration increase.

In another apparatus configuration, the apparatus does not include a concentrator module, but includes a preparation module adapted for preparing a concentrated electrolyte by combining a concentrated copper salt and a concentrated acid. This configuration is illustrated in FIG. 7, and is suitable for performing a method shown in FIG. 2B. The apparatus includes a reservoir 703 which is adapted to receive a concentrated solution of copper salt through inlet port 799 from the source of concentrated copper salt 791. The flow of concentrated copper salt is controlled by the valve 795. The reservoir 703 also includes an inlet port for receiving concentrated acid solution from the source of concentrated acid 793, where the flow of acid is controlled by a valve 798. The concentrated solutions of copper salt and acid are mixed in the reservoir 703 to form a solution that would have been fully saturated at 0° C., or, in some embodiments, fully saturated at 20° C. The temperature in the reservoir is controlled such that the formed electrolyte remains fully in solution. For example in some embodiments, the electrolyte is maintained at a temperature of between about 20-35° C. In some embodiments, it is preferable to maintain the electrolyte at a temperature of at least about 40° C., such as at a temperature of between about 40-65° C. The reservoir will typically include an immersion heater 719 and temperature detectors connected with the controller unit 725 which is adapted to control the temperature in the reservoir. The reservoir may also include a concentration detector (not shown) connected to the controller 725. Similarly to the reservoir depicted in FIG. 6, the reservoir 703 includes an inlet port 773 adapted for receiving electrolyte additives from an additive source 713, controllable by valve 771. The reservoir also includes an emergency overflow conduit 775, and an overflow shutoff valve 767 connected to member 761, which is adapted to close the delivery of the diluent at diluent port 765 from the diluent source 711. The diluent flow can also be controlled by valve 769. The concentrated electrolyte from the reservoir 703 is directed to the plating cell 705 to contact the

substrate 759. The plating cell in this embodiment is configured similarly to the plating cell described in FIG. 6

#### Example

In one illustrative example, a solution containing copper sulfate at  $\text{Cu}^{2+}$  concentration of between about 65-85 g/L is directed from source 791 to the reservoir 703. The solution in the reservoir is heated to a temperature of about 35° C., and then sulfuric acid having a concentration of between about 900-1800 g/L is added to the reservoir and is mixed with the solution of copper sulfate to form a concentrated solution having 60-80 g/L  $\text{Cu}^{2+}$  and between about 5-50 g/L sulfuric acid. The resulting concentrated solution is directed to the plating cell 705, where copper is electrodeposited on the substrate at a temperature of about 30-35° C.

Although various details have been omitted for clarity's sake, various design alternatives may be implemented. Therefore, the present examples are to be considered as illustrative and not restrictive, and the invention is not to be limited to the details given herein, but may be modified within the scope of the appended claims. For example, in some embodiments, the concentrator module need not be necessarily a separate unit connected with the reservoir by tubing, but may reside physically within the reservoir. In other embodiments, the reservoir is not used in the apparatus configuration, and the concentrated electrolyte solution is flowing directly from the concentrator module into the plating cell. Yet in other embodiments, the concentrated electrolyte is prepared from copper salt and acid within the lines connected to the plating cell, without having a separate reservoir for mixing. Suitable temperature of the electrolyte can be achieved partially or fully due to exothermic mixing of concentrated acid solution with the solution of the salt.

The controller associated with the apparatus can include program instructions for performing any of the methods provided herein. In some embodiments the controller is used and has program instructions to automatically dilute the concentrated electroplating solution, when it is determined that the concentrated solution is at risk of forming a precipitate, or when the precipitation has started. In some embodiments the controller is used and has program instructions to automatically remove some or all of the concentrated electroplating solution from a vessel to a drain, when it is determined that the concentrated solution is at risk of forming a precipitate, or when the precipitation has started. In other embodiments the controller is used and has program instructions to automatically remove a portion of the concentrated electroplating solution from a vessel to a drain and to add an appropriate amount of a diluent (e.g. water) to the vessel and/or drain so that the resultant concentrations of electrolyte components in the vessel and in the drain are such that the electroplating solution remains soluble at ambient temperature. These actions are triggered when it is determined that the concentrated solution is at risk of forming a precipitate of a salt, for example, due to a drop in measured solution temperature below a preset limit, or when the precipitation is detected (e.g., by a particle sensor), or when a precipitation-related parameter (e.g., density and conductivity measured in the solution) indicates that the concentrations of the solution components are near the solubility product or at the solubility product of the salt at the temperature measured in the vessel.

Precipitation of metal salts from concentrated solutions (e.g., due to an inadvertent temperature drop) is a serious risk that can result in the disruption of electroplating process and in damage of the electroplating equipment (e.g. damage

to the pumps, membranes and housing of the electroplating cell). The provided dilution and/or solution disposal control can be applied to one or more vessels described herein that are configured to contain a heated concentrated electrolyte, and to any combination of such vessels. For example, this type of control can be applied to the electroplating cell itself (such as the cells 605 and 705 shown in FIGS. 6 and 7 respectively), to a reservoir holding the heated concentrated electrolyte (such as reservoirs 603 and 703 shown in FIGS. 6 and 7 respectively), to a concentrator, where the concentrated electrolyte is generated from a dilute electrolyte (such as in the concentrator 601 shown in FIG. 6), and, in some cases, to fluidic delivery lines or drain lines (when the concentrated hot electrolyte is generated, disposed of, or stored in lines). The vessel to which this control is applied is generally in fluidic communication with an electroplating cell, or the vessel itself is the electroplating cell.

In one implementation, the vessel, equipped with such dilution and/or solution disposal control is configured to maintain a concentrated electroplating solution at a temperature of at least about 40° C., wherein the solution would have formed a precipitate at a lower temperature such as at 0° C. or at 20° C. (i.e. the electrolyte is “supersaturated” at these temperatures). The vessel can be any of the vessels described above and is generally in fluidic communication with the electroplating cell, or the vessel itself is the electroplating cell. In some embodiments this vessel includes a heater configured to heat the concentrated solution to a temperature at which the solution is fully soluble; in other embodiments the heater may not be needed due to influx of fresh hot solution into the vessel or due to an exothermic reaction (e.g., due to exothermic mixing of concentrated acid and water) within the vessel. The heater can be an immersion electrical heater, or a heat exchanger (e.g., shell and tube, or immersion coil, coupled with an external heat source or heated circulating fluids). The apparatus further includes a controller having program instructions for adding a diluent to the concentrated electroplating solution in the vessel and/or opening the drain and removing some or all of the electrolyte from the vessel to avoid precipitation of a salt from the concentrated electroplating solution in response to a signal. For example, the user of the apparatus can determine that if the temperature of the electroplating solution in the vessel drops below a certain value (where the value is referred to as “desired temperature”, or a minimum safe temperature control limit) the electroplating solution is at risk of forming a precipitate. Similarly, the apparatus user can determine that if a concentration of one or more components in the electroplating solution rises above a certain level (where the level is referred to as “desired concentration” or maximum safe concentration control limit), a precipitation of salts may occur.

The apparatus further includes one or more sensors configured to monitor a property of the concentrated electroplating solution that is related to precipitation (possible or already occurring) of a salt from solution. The measured properties related to precipitation include temperature and concentration of electrolyte components in solution (where concentration measurements includes measurement of parameters that correlate with the concentration, such as optical density, density, and conductivity of the concentrated solution). For example, temperature is a precipitation-related property because the solubility product of the salt depends on the temperature, and precipitation can be triggered by a drop in temperature. The density of solution is a precipitation-related property because it correlates with the concentration of metal salt in solution, and an increase in

density may indicate that the solution is at risk of precipitation. Measurement of the concentrations of the solution components (via measurement of concentration-correlating parameters) can be made by various inline or in-situ metrology sensors, including but not limited to ion-selective electrodes, rotating disc limiting current sensors, optical absorption sensors, Raman spectroscopy sensors, densitometers, viscosity meters, conductivity meters, and automated titrators. In one of the preferred embodiments, in a continuous in situ method for determining concentrations of components in a solution comprising a single salt of a metal and an acid having the same anion as the metal salt, a densitometer and a conductivity meter are used together as sensors. The densitometer measures the density of the solution which strongly correlates with the concentration of metal ions in the solution, while the conductivity meter measures the conductivity of solution, which strongly correlates with the concentration of acid in the solution (and with the amount of the common anion in solution). Taken together, with knowledge of the relationship between metal and acid concentration dependencies on density and solution conductivity, these sensors allow one to determine the metal and acid concentrations in solution continuously and accurately. These sensors may send the measured parameters to the controller, which is configured for processing the parameters and determining if the concentrations of acid and metal salt exceed the desired value in the vessel. If the concentrations are exceeded, the controller provides a signal for dilution of the solution in the vessel and/or for removal of a portion or all of the solution from the vessel. For example if the vessel operates at an operation temperature of 20 or 25 degrees C., and it originally contained a solution that would have formed a precipitate at 0 degrees C., the controller can be triggered with a signal for dilution if the concentrations of components in the electroplating solution increased to a level that is near or at the solubility product of the salt at the operating temperature (i.e., the solution is at a risk of precipitation or the precipitation has started).

The appropriate or best forms of measured parameters and their dilution-triggering or removal-triggering values can be readily determined by one of skill in the art for different types of electrolytes and may be provided to the controller in the form of program instructions. As it was mentioned above, one or more sensors in the vessel are configured to measure the temperature of the concentrated electroplating solution and/or the concentrations of components (in the form of parameters correlating with concentrations) of the electroplating solution (e.g., copper salt concentration and/or acid concentration). The sensors will provide a signal related to these parameters which can be manually or automatically (e.g., through electrical communication) transmitted to the controller. If the signal provided by the sensor or sensors indicates that the temperature of the electroplating solution dropped below the desired value programmed into the controller (e.g., due to a failure of the heater, inefficient electrolyte mixing, high rate of evaporation or failure of the system to handle water makeup associated with evaporation etc.), the controller will instruct the apparatus to inject a diluent (e.g., deionized water) into the vessel in order to avoid precipitation of the metal salts. In some embodiments the amount of added diluent is calculated by the controller such that it is sufficient to avoid precipitation. In some embodiments, a portion of the concentrated electrolyte is removed from the vessel prior to and in conjunction with the dilution. This may be needed if the vessel does not have sufficient volume to contain the necessary amount of diluent. In some embodiments a portion of

the concentrated electroplating solution is removed from the vessel through drain lines and the controller is further programmed to provide diluent to the drain lines in order to avoid precipitation of the metal salts in the drain. In other embodiments (where sufficient volume is available) the solution in the vessel is diluted to a concentration where precipitation would not occur at 20° C. and then the volume of the solution is returned to the original, lower volume by passing the electrolyte that is stable at 20 degrees C. (does not form precipitate at 20 degrees C.) to the drain.

In one of the embodiments, the dilution control is applied to the apparatus illustrated in FIG. 7. In this embodiment the concentrated electroplating solution is formed in the reservoir 703 by providing a concentrated metal salt solution (e.g., copper salt solution) from a source of concentrated metal salt 791, heating the metal salt solution and by then adding concentrated acid from a source of concentrated acid 793 and thereby forming the concentrated solution that would have formed a precipitate at 20 degrees C. or, in some embodiments at 0 degrees C. In an alternative embodiment, the same solution can be formed when the concentrated metal salt is added to the solution of concentrated acid first provided to the vessel. In some embodiments, the concentrated metal salt at the source also contains acid in low amount, and is fully soluble at a reduced temperature (e.g. -5° C., or 20° C.). The source of concentrated metal salt may include a commercially available concentrated metal salt solution in a tank. Alternatively, the concentrated metal salt solution can be generated on site. In one embodiment, the source of concentrated metal salt includes a concentrator that is configured to generate a concentrated solution from a more dilute solution via evaporation of water or reverse osmosis. In another embodiment, the source of concentrated metal salt solution includes an electrochemical generator, where the solution is generated using electrochemical dissolution of a metallic anode (e.g., copper anode). Such generator is described, for example, in the commonly owned U.S. Provisional Application Ser. No. 62/168,198 by Mayer et al. filed on May 29, 2015 and titled "Electrolyte Delivery and Generation Equipment", which is herein incorporated by reference. In some embodiments the reservoir where mixing of concentrated metal solution and concentrated acid takes place is equipped with a sensor (e.g., a temperature sensor and/or a concentration sensor, such as those described above, e.g., a densitometer and a conductivity meter) that communicates signals to a controller. If the controller receives the signal that the temperature has dropped below a desired value and/or the concentration of metal salt rose above a desired value, the controller provides instructions for adding a diluent (e.g., water) to the reservoir and/or for removing a portion or all of the electroplating solution from the reservoir through a drain. In a modification of this embodiment, the concentrated metal salt solution is mixed with the concentrated solution in lines before it is delivered to the reservoir and/or electroplating cell. Any one of the delivery lines, the reservoir, and the electroplating cell can be a vessel equipped with a dilution control as described herein.

In some embodiments, the reservoir and the cell are not separate elements and the solution in the cell-reservoir vessel is maintained at a temperature of at least about 40 degrees C. as described above and the apparatus is configured for dilution and/or draining using a controller, as described above.

In some embodiments a method of dilution-based control against precipitation is provided, wherein the method involves providing a diluent (e.g., water) to a vessel con-

taining a concentrated electroplating solution, (e.g., a solution that would have formed a precipitate at 20° C., or a solution that would have formed a precipitate at 0° C.) when it is determined that the solution is at a risk of precipitation. 5 In some embodiments, a sensor or sensors measure the temperature of the concentrated electroplating solution in the vessel and/or concentration of metal salt in the vessel (via measurement of concentration-related parameters described above) and send these parameters to a controller 10 having program instructions to dilute the electroplating solution in response to a selected signal (e.g., when the temperature is below a desired temperature or the concentration of one or more components is above the desired concentration). The method may also involve removing a 15 portion of concentrated electroplating solution from the vessel in conjunction with addition of diluent into the vessel. A diluent may also be added to the drain lines as the electroplating solution is removed through the drain lines. In an alternative embodiment, the concentrated electroplating 20 solution is completely removed from the vessel in response to the signal indicating that the solution is at risk of precipitation or has started forming a precipitate. In this case a diluent may be added to the drain line.

What is claimed is:

1. An electroplating apparatus for depositing a metal on a semiconductor substrate having one or more recessed features, the apparatus comprising:

(a) a vessel configured to maintain a concentrated electroplating solution at a temperature of at least about 40° C., wherein said solution would have formed a precipitate at 20° C.;

(b) an electroplating cell configured for bringing the concentrated electrolyte in contact with the semiconductor substrate at a temperature of at least about 40° C., wherein the vessel is in fluidic communication with the electroplating cell or wherein the vessel is the electroplating cell;

(c) one or more sensors, configured to monitor one or more properties of the electroplating solution related to precipitation of a salt from the electroplating solution in the vessel, wherein the one or more sensors comprise a sensor selected from the group consisting of a temperature sensor and an optical concentration sensor, and are in communication with an apparatus controller; and

(d) the apparatus controller comprising program instructions for:

(i) receiving readings provided by at least one of the temperature sensor and the optical concentration sensor;

(ii) causing a generation of a signal if temperature drops below a pre-determined value or if a concentration of the metal salt determined by the optical concentration sensor rises above a pre-determined value, wherein said pre-determined values are indicative of a risk of metal salt precipitation and are pre-set in the controller; and

(iii) causing an addition of a predetermined amount of a diluent to the concentrated electroplating solution in the vessel in response to the signal to avoid precipitation of the salt from the concentrated electroplating solution in the vessel.

2. The electroplating apparatus of claim 1, wherein the one or more sensors comprise a temperature sensor.

3. The electroplating apparatus of claim 1, wherein the one or more sensors comprise a temperature sensor and an optical concentration sensor.

## 27

4. The electroplating apparatus of claim 1, wherein the vessel is a concentrated electrolyte reservoir in fluidic communication with the electroplating cell.

5. The electroplating apparatus of claim 4, wherein the vessel is in fluidic communication with a source of concentrated metal salt and with a separate source of concentrated acid.

6. The electroplating apparatus of claim 5, wherein the apparatus controller further comprises program instructions for:

- (iv) causing an introduction of the concentrated solution of metal salt to the concentrated electrolyte reservoir and causing a heating of the concentrated solution of metal salt in the concentrated electrolyte reservoir; and
- (v) causing mixing of the heated concentrated solution of metal salt with the concentrated acid to obtain the concentrated electroplating solution.

7. The electroplating apparatus of claim 5, wherein the apparatus comprises a source of concentrated metal salt in fluidic communication with the vessel, wherein the source of concentrated metal salt comprises a concentrator tank that is configured to generate a more concentrated metal salt solution from a dilute metal salt solution.

8. The electroplating apparatus of claim 5, wherein the apparatus comprises a source of concentrated metal salt in fluidic communication with the vessel, wherein the source of concentrated metal salt comprises a generator that is configured to electrochemically produce a concentrated metal salt solution using electrochemical dissolution of a metallic anode.

9. The electroplating apparatus of claim 5, wherein the apparatus comprises a source of concentrated metal salt in fluidic communication with the vessel, wherein the source of concentrated metal salt is a tank filled with concentrated metal salt solution.

10. The electroplating apparatus of claim 1, wherein the controller further comprises program instructions for causing a removal of a portion of the concentrated electroplating solution from the vessel in conjunction with diluting the concentrated electroplating solution in the vessel.

11. The electroplating apparatus of claim 1, wherein the vessel is a concentrator vessel, configured to generate a concentrated electroplating solution from a dilute electroplating solution.

## 28

12. The electroplating apparatus of claim 1, wherein the vessel is the electroplating cell, configured to hold the semiconductor substrate in contact with the hot concentrated electroplating solution.

13. The electroplating apparatus of claim 1, wherein the vessel comprises a heater.

14. The electroplating apparatus of claim 1, wherein the optical concentration sensor is an optical absorbance sensor.

15. An electroplating apparatus for depositing a metal on a semiconductor substrate having one or more recessed features, the apparatus comprising:

- (a) concentrated electrolyte reservoir configured to maintain a concentrated electroplating solution at a temperature of at least about 40° C., wherein said solution would have formed a precipitate at 20° C.;
- (b) an electroplating cell configured for bringing the concentrated electrolyte in contact with the semiconductor substrate at a temperature of at least about 40° C., wherein the concentrated electrolyte reservoir is in fluidic communication with the electroplating cell, with a source of concentrated metal salt, and with a separate source of concentrated acid;
- (c) one or more sensors configured to monitor one or more properties of the electroplating solution related to precipitation of a salt from the electroplating solution in the concentrated electrolyte reservoir, wherein the one or more sensors are in communication with an apparatus controller; and
- (d) the apparatus controller comprising program instructions for:
  - (i) causing an introduction of the concentrated solution of metal salt to the concentrated electrolyte reservoir and causing heating of the concentrated solution of metal salt in the concentrated electrolyte reservoir;
  - (ii) causing mixing of the heated concentrated solution of metal salt with the concentrated acid to obtain the concentrated electroplating solution and
  - (iii) causing a diluent to be added to the concentrated electroplating solution in the concentrated electrolyte reservoir in response to a signal originating from the one or more sensors to avoid precipitation of the salt from the concentrated electroplating solution in the vessel.

\* \* \* \* \*